

## UNITED STATES PATENT OFFICE

2,018,758

LUBRICATING COMPOSITION AND PROCESS  
FOR MAKING THE SAMECarleton Ellis, Montclair, N. J., assignor to  
Standard Oil Development CompanyNo Drawing. Application May 3, 1932,  
Serial No. 609,038

13 Claims. (Cl. 87—9)

The present invention relates to improved lubricating oils particularly those of high lubricating value of the petroleum type, and relates especially to an improved method for producing such oils by the addition of substances which even when present in relatively small proportions exert a beneficial influence of an unexpected character. My invention will be fully understood from the following description of the product and its method of manufacture.

Various addition agents have been incorporated from time to time in lubricating oils for the purpose of increasing their load bearing capacity or for other similar reasons. I have found, however, that many of these agents while extremely effective for some particular combination of bearing metals are not equally desirable for other types of bearing combinations. The present invention is concerned with a class of substances possessing a property of notable significance, i. e., that of imparting to the lubricant a higher degree of film strength in substantially all types of bearing combinations or, if in certain bearing metal combinations it is not substantially raised, at least it may be said that the presence of these substances does not lower the film strength for such bearing metal combinations, while other properties obtain as hereinafter disclosed. By this means the film strength generally is perceptibly increased permitting the use of smaller bearing surfaces and enabling the journals or other types of bearings to be operated under more severe conditions of load, speed and the like. The compounds of this sort which are disclosed below thus favorably affect the state of tension of the lubricating film and may be termed tensionizers.

Another valuable property of many of the materials disclosed below is that they act as pour inhibitors. Lubricating oils produced from crude oil, hydrogenated hydrocarbon oils and the like contain waxy constituents in such amounts as to cause the oil to congeal or solidify at relatively high temperatures within the range in which such oils could otherwise be used as lubricants. Oils from paraffin or mixed base crudes in many cases solidify at 50 or even 75° F. for the heavier cuts and the lighter distillates often solidify as high as 30 or 40° F.

It is the practice in modern refineries to remove at least a portion of the wax so as to reduce the solidification point to 25, 20 or 0° F. or even lower. Waxy hydrocarbons are generally removed by filtration at reduced temperatures, or by similar methods such as cold settling or

centrifugal means, but all of these methods require expensive refrigeration.

On the other hand, the invention is likewise applicable to oils which have not been dewaxed or oils to which, for one reason or another, paraffin wax, ceresin wax, petrolatum and the like, has been added.

As stated above many of the substances disclosed below act not only in the capacity of tensionizers but likewise exert a pour inhibiting influence. Therefore, according to the preferred form of my invention I utilize compounds which are capable of functioning in the dual role of pour depressant and tensionizer and which may be designated as pour depressant tensionizers or tensionizing pour depressants.

The materials which form the basis of my invention are nitrogen-containing and of the class formed by the reaction of hydroxy amines, particularly the alkyloamines such as methanol-, ethanol-, propanol-, butanol- and the higher hydroxy amines with an organic acid, specifically the esters formed thereby which are adequately soluble in petroleum lubricating oils to function in the manner described above. I do not wish to exclude, however, as pour depressants and/or tensionizers the salts of the amines such as formed by the simple addition of the acid to the amine and which reaction is characterized by combination without elimination of water; preferably, the products which fall within certain specific confines of the present invention are the true esters formed by the reaction of acids with hydroxy amines and characterized by the elimination of water. In such cases amine salts, if desired, may be present, or the product may at the same time be an amine salt and amino ester.

The said products may be obtained in the same manner in which true esters are formed, for example, by mixing the alcoholic material, that is to say, the hydroxy amine in this instance, with the organic acid and effecting the esterification, for example, in the presence of sulphuric acid or other inorganic acids in the ordinary, well-known manner, or the esterification may be accomplished by heating the reactants at a temperature of 212° F. or somewhat higher in the absence of mineral acids. Those methods are apt to produce a certain amount of the salt as well as the ester and if it is desired to produce only the ester, 3 mols of the acyl chloride may be heated with, for example, 1 mol of the trihydroxy amine in the presence of a basic material such as pyridine. In such case the hydrochloride of pyridine is formed, and the ester of the hydroxy amine and

organic acid is produced without any substantial quantity of salt. This particular method, however, forms no part of the present invention.

For my purposes I prefer to use the poly-  
5 hydroxy amines, chiefly the trihydroxy amines, although the lower hydroxy amines, particularly the aliphatic hydroxy amines may be used insofar as solubility permits. For example, the tri-  
10 ethanol amine of commerce which generally stock for my purpose.

With regard to the acid radicals, I prefer the higher fatty acids, that is to say, the acids in the  
15 range of stearic, oleic and the like, and particularly I prefer the higher acids derived from paraffin wax by low temperature oxidation. These latter acids may be produced, for example, by oxidation with strong nitric acid, or by blowing  
20 air or other oxidizing gases through molten paraffin, first at temperatures corresponding to the melting point of wax or somewhat higher and, preferably, in the presence of catalysts such as the previously oxidized wax, manganese and cobalt resins, barium cinnamate and the like, mixtures of these materials or other appropriate catalysts. The naturally occurring acids such as stearic, oleic, behenic or erucic may be used  
25 as well as the heavier unsaturated acids or mixtures of these various materials.

These esters may be dispersed through the wax containing hydrocarbon oil by means of a solvent, as for example alcohol, benzene, naphtha, or any other similar light solvent capable of dissolving  
30 the esters and mixing with the waxy oils. The solution of the ester is added to the wax-containing oil which is then thoroughly agitated to form a homogeneous mixture after which the temperature of the mixture may be raised to such a degree as to boil off the low-boiling solvent without decomposing the heavier oil. If preferred the solvent may be eliminated altogether, and the ester mixed with the oil, preferably by heating to about 300° F. Or the ester may be added to a portion of the oil thus forming concentrates which can be used advantageously as additions to the oil stock in suitable proportions.

The ester may be added to the oil in any desired proportion, for example, below 10 per cent or 5 per cent. The different substances vary somewhat in their pour inhibiting and/or tensionizing powers and consequently will be used in somewhat different proportions; often about 1 to 2 per cent is the most desirable. There is generally an optimum quantity for pour inhibiting strength; for instance, if too little of the pour inhibitor is used the maximum pour reduction is not obtained, and at the same time if too great a quantity is used qualities of the oil may be altered to a degree undesirable for the particular purpose in hand. In general it may be said that the optimum quantity is nearly always within the range from about 0.1 to 10 per cent, and the proper quantity of ester required for a particular oil can be readily determined by test.

As an example of the action of substances made according to my invention the following may be taken as illustrative. The tensionizing pour inhibitor is made in the manner described above from triethanolamine and a mixture of acids obtained by the oxidation of paraffin wax by blowing with air at temperatures of about 200° to 300° F. The triethanolamine and the acids are used in the proportion of 1 of the amine to about

3 of the acid, that is in stoichiometric proportions, and esterification is carried out at an elevated temperature. This material is added to an engine oil of the following specifications:

Gravity, 30.6° A.P.I.

Viscosity (Saybolt) at 100° F., 150 seconds.

Viscosity (Saybolt) at 210° F., 45 seconds.

Pour, 30° F.

Flash, 395° F.

Color (Robinson), 10%.

When the proportion of ester added was 0.5 per cent it was found that the solidification point of the oil, 30° F., was reduced to 15° F. When the pour inhibitor was added in the proportion of about 2 per cent to the same oil, its pour point 15 was reduced to -5° F. In both cases the other above mentioned properties of the oil were substantially unchanged. The load bearing capacity of the blended oil was tested in respect to various different bearing combinations by the Mougey 20 method as described in the National Petroleum News, November 11, 1931, page 47. The following bearing combinations were used:

Steel to bronze.

Steel to aluminum.

Steel to Babbitt.

Steel to cast iron.

Cast iron to cast iron.

Cast iron to aluminum.

Steel to steel.

In all of these cases the blended oil gave excellent service.

While, as has been indicated, different metal bearing combinations afford differing degrees of service, it may be noted that in the case of steel 35 to aluminum, cast iron to aluminum and steel to steel, the oil with tensionizer aforesaid gave considerably better service than the untreated oils. In using larger amounts than 2 per cent the pour inhibiting power was somewhat dim- 40 finished. It is possible however to establish simultaneously in a given oil adequate tensionizing and pour inhibiting proportions of the active amino compound.

The pour inhibitor or pour depressant and/or tensionizer may be prepared also simply by heating the amine and organic acid together without sulphuric acid or other strong acid catalyst of esterification. This step if desired may be carried out in the oil itself or in a portion of the oil. 50 In the latter case a concentrate can be prepared similar to that indicated above. Oil which is at a high temperature from some other previous operation may receive additions of the components of the pour depressant and/or tensionizer, 55 illustratively the acids from oxidized paraffin wax and triethanolamine, reaction taking place in the hot vehicle and deriving the product in a very convenient manner.

On the other hand the pour depressant or tensionizer may, for example, in the absence of an oil diluent such as that mentioned above, be further concentrated if necessary to a higher degree of potency by treatment with appropriate solvents to separate and remove inactive or less active components.

It should be mentioned also that with hydroxy amines containing two or more hydroxyl groups in the molecule (polyhydroxy amines), such as triethanolamine, I may also make esters by mixing the amine and fatty acids in the stoichiometric proportions of 1 part of amine to 1 part of acid, or 1 part of amine to 2 parts of acid, instead of the ratio of 1 part of amine to 3 parts of acid as given in the above example. Furthermore

crude acids obtained by the oxidation of paraffin wax may be fractionated, for example by means of vacuum distillation and a low boiling or higher boiling fraction used, ranging from liquid or soft acid material to hard wax acids, as desired. In general the compounds comprised herein preferably are derived from higher fatty acids and the like including those the molecule of which contains 10 carbon atoms and over. Wax acids 10 embrace a wide range of acids as denoted by the number of carbon atoms, whereas the acids derived from animal and vegetable fats possess carbon atoms from say 12 to 22 in number, the acids commonly available being those of 12, 16, and 18 15 carbon atoms. These various fatty acids are comprised under the term "higher fatty acids" as used in the foregoing.

In addition to the foregoing additions to lubricating oils in accordance with the preferred form 10 of my invention I also may add anti-oxidants such as certain bodies containing phenolic groups. Certain amino compounds also act as anti-oxidants and the amino compounds included in the present invention serve for this purpose to 25 the extent that such function is available, but others may be added for additional effect. The addition of these substances may be made to an oil which has been used so as to become slightly oxidized and is susceptible to further oxidation 10 accompanied by sludge formation. These materials not only reduce the susceptibility of the oil to further oxidation but also modify the oil by imparting to it a greater load bearing capacity and pour reducing properties as indicated above.

15 My process serves as a valuable aid in the recovery of used lubricating oils. After considerable heavy service a lubricating oil develops acidity and sludge. The sludge may be removed in a variety of different ways, for example by filtration which also removes metal particles and dirt; sludgy constituents which are not entirely removed by filtration can be removed by adsorptive means such as by the use of fuller's earth and the like. These methods will leave the oil, however, in an acid condition. If desired I may add my alkylolamines directly to this oil in the preferred proportions and the oil may be heated at an elevated temperature so as to cause combinations between the acids of the oil and these 10 added substances. In this way the alkylolamines serve as purifying agents for the oil in eliminating acidic bodies and at the same time converting them into substances which give additional valuable properties to the oil.

20 My oils, whether originally produced by the addition of the alkylamine esters, acids or the like to fresh hydrocarbon oils, or whether present in the oil due to recovery of the used lubricating oil, find a valuable application as "breaking-in" 25 oils. For this purpose the oil is used in the ordinary manner for the first 500 to 1000 miles of operation in a new car. As is well known the bearings of the car are not completely worn in and due to tool marks and high spots there is ordinarily a considerable danger of seizure, scoring and other equally bad effects. However, my oils which contain the tensionizers are endowed with a sufficiently high film strength to almost completely eliminate any of the dangers enumerated 30 above and when such an oil is used it is proposed to operate a new car from the start at relatively high speeds and to disregard the usual care during the "breaking-in" period.

35 In like manner these pour depressants may be incorporated in greases or gear oil such as trans-

mission grease to aid in reducing the tendency to channelling and the like.

In the above description I have mentioned generally all types of combinations of the alkylolamines with fatty or other organic acids. While all of these materials bring about improvements in lubricating qualities, I have observed that the true esters are more soluble and more desirable than either the salts or the ester salts, that is to say, the materials which are both esters and salts. For this reason I have a marked preference for the esters alone. Not only are they superior in respect to tensionizing influences but also their pour reducing properties are markedly superior.

15 My invention is not to be limited by any theory of the mechanism of pour reduction or of "breaking-in" nor to the particular substances described for purposes of illustration, but only to the following claims in which I wish to claim all novelty 20 inherent in my invention.

I claim:

1. A composition of matter comprising a mineral lubricating oil containing an organic product of the reaction of an organic acid with an 25 alkylol group of an alkylolamine.

2. A mineral oil containing a minor quantity of an organic reaction product of an organic acid containing at least 10 carbon atoms with an alkylol group of an alkylolamine.

3. A mineral oil according to claim 2 in which the organic acid has from 10 to 22 carbon atoms.

4. An oil according to claim 2 in which a polyalkylolamine is used.

5. A lubricating oil comprising a mineral oil 35 and a minor quantity of an ester produced by the reaction of an alkylolamine and an organic acid.

6. A mineral oil according to claim 5 in which the ester is produced from a polyalkylolamine.

7. An improved lubricating oil comprising a 40 viscous hydrocarbon oil containing a minor proportion of an ester of a trialkylolamine and an organic acid of at least 10 carbon atoms.

8. An improved lubricating oil comprising a viscous hydrocarbon oil containing an ester produced by the reaction of triethanolamine and an organic acid of at least 10 carbon atoms, said ester being in tensionizing and pour inhibiting proportions.

9. An improved lubricating oil comprising a 50 viscous waxy oil and an organic product of the reaction of an organic acid having at least 10 carbon atoms with an alkylol group of a polyalkylolamine in tensionizing and pour reducing proportions.

10. An improved lubricating oil comprising a viscous hydrocarbon oil containing waxy constituents, and an ester formed by the reaction of a polyalkylolamine and an organic acid containing at least 10 carbon atoms, said ester being in 60 tensionizing and pour reducing proportions.

11. Lubricating oil composition comprising a viscous waxy oil containing in a dissolved state an organic product of the reaction of an alkylolamine with an organic acid having at least 10 65 carbon atoms in pour reducing proportions.

12. Lubricating oil composition comprising a viscous waxy hydrocarbon oil containing in a dissolved state an organic product of the reaction of a polyalkylolamine with a fatty acid of at least 70 ten carbon atoms in a pour reducing proportion of not more than about two per cent.

13. A mineral oil composition according to claim 5 in which said organic acid is a fatty acid.

CARLETON ELLIS. 75